

July 10, 1956

R. A. WILKINS ET AL.

2,754,196

## METHOD OF ELECTROTHERMICALLY SMELTING ZINC

Filed April 12, 1951

4 Sheets-Sheet 1



inventors  
Richard A. Wilkins  
Kenneth A. Phillips  
DyEmery Ruth Townsend Miller  
W. Weidner

July 10, 1956

R. A. WILKINS ET AL

2,754,196

METHOD OF ELECTROTHERMICALY SMELTING ZINC

Filed April 12, 1951

4 Sheets-Sheet 2

*Fig. 2*



Inventors:  
Richard A. Wilkins  
Kenneth C. Phillips  
By Harry Booth Townsend Miller  
Weldner  
Attest:

July 10, 1956

R. A. WILKINS ET AL

2,754,196

## METHOD OF ELECTROTHERMICALLY SMELTING ZINC

Filed April 12, 1951

4 Sheets-Sheet 3

Fig. 3



Fig. 6



Inventors  
Richard A. Wilkins  
Katherine A. Phillips  
Dorothy B. Townsend Miller  
Wieder Clegg

July 10, 1956

R. A. WILKINS ET AL

2,754,196

## METHOD OF ELECTROTHERMICALLY SMELTING ZINC

Filed April 12, 1951

4 Sheets-Sheet 4



Investors  
Richard A. Watkins  
Kenneth A. Phillips  
Emery Booth Townsend Miller  
J. Weidner  
Otis, S.

2,754,196

**METHOD OF ELECTROTHERMICALLY  
SMEILING ZINC**

Richard A. Wilkins, Rome, N. Y., and Kenneth A. Phillips, Collinsville, Ill., assignors to Revere Copper and Brass Incorporated, Rome, N. Y., a corporation of Maryland

Application April 12, 1951, Serial No. 220,574

7 Claims. (Cl. 75—14)

Our invention relates to methods of smelting zinciferous materials, containing zinc oxide, by heating them in the presence of carbon to react the zinc oxide with the carbon whereby to liberate metallic zinc. The invention also relates to furnaces and apparatus comprising the same capable of, among other uses, being used in the practice of such methods.

The invention has among its objects an increased recovery of zinc from the zinciferous material treated, the provision of a loose charge enabling a continuous smelting operation to be readily effected, and, when desired, the simultaneous recovery with the zinc of a matte containing the precious metal values of the zinciferous material. These and other objects of the invention will be best understood from the following description of several forms of the method and apparatus according to the invention, while the scope of the invention will be more particularly pointed out in the appended claims.

Commonly the significant zinciferous content of zinc ore as mined is zinc sulphide. After being mined the ore is crushed and subjected to a separating operation for removing as much of the gangue as economically feasible. The resulting zinc ore concentrate is then roasted in the presence of air for converting the zinc sulphide to zinc oxide. Commercially the resulting product is commonly known as "zinc sinter" or "zinc calcine," depending upon the exact roasting method employed, the "sinter" being more or less fused as distinguished from the "calcine." Both, however, are granular materials or may readily be made such by subjecting them to a slight crushing operation. Generically these products are herein sometimes referred to as "oxidized zinc ore" in conformity with the terminology commonly employed in the smelting industry.

The oxidized zinciferous material produced by the above mentioned roasting operation contains some of the gangue of the original ore, which gangue is largely silica or other fusible substance capable of slagging if heated to the requisite temperature, the melting point of the slag being about 1950 to 2250° F. depending upon its exact composition. Also this oxidized zinc ore contains other impurities among which is practically always iron in the form of iron oxide and usually some iron in the form of iron sulphide, both of which may readily be reduced to produce metallic iron by heating the oxidized zinc ore in the presence of carbon, such iron because of its carbon and silicon content being liquid at the temperature of the liquid slag. In most instances the oxidized zinc ore further contains a small amount of copper in the form of sulphide, usually with some oxide or other copper bearing compound or mineral which will form copper sulphide when the oxidized zinc ore is heated in the presence of carbon and the residual zinc sulphide in the zinc ore and sulphur in the coke or coal supplying the carbon. Also the oxidized zinc ore commonly contains a small but economically valuable amount of the precious metals gold and silver.

According to the present invention, the oxidized zinc

ore containing the zinc oxide and impurities is mixed in granular form with reaction carbon in granular form and the mixture charged to a hearth in an operatively closed chamber to form on the hearth a mass of the charge having an upper downwardly sloping free surface which at its lowermost portion is substantially in the plane of the hearth. This reaction carbon preferably is in the form of coke or anthracite coal rendered granular by a crushing or grinding operation, or "coke breeze," or bituminous coal "fines." In the particular forms of apparatus illustrated by the drawings the mixture is fed to the chamber from below the sloping surface of the mass of charge and adjacent its higher portion so that the charge being fed forces the material of the mass to this sloping surface substantially throughout its entire extent and thus also acts to move away from the body of said mass the material of the mass adjacent the lower edge of said sloping surface, the slant of this sloping surface being largely determined by the angle of repose of the granular charge. Feeding the material to the mass in this way causes it to be preheated when it reaches the sloping surface of the mass as hereinafter more fully explained, and thus avoids any necessity of preheating the charge exteriorly of the chamber preliminarily to entering it thereinto as would be the case if the charge were fed to the chamber from above said sloping surface and it were desired to enter it in preheated condition. Heat is radiated downward on said sloping surface to heat the surface portion of the mass of charge to a temperature which will react the zinc oxide with the carbon and melt the slag forming materials of the oxidized zinc ore and of the coke or coal of the charge. This heat also is sufficient to react with the carbon at least some of the iron oxide present, and some of any iron sulphide present, at the surface portion of the mass so as to produce molten iron as well as molten slag, the copper sulphide dissolving into the iron so that the iron significantly is in the form of an iron-copper matte mixture. This iron also contains dissolved carbon and commonly silicides which act to reduce its melting point. Such molten slag and iron so produced adhere as more or less viscous droplets to solid particles of excess coke or coal and to other solid particles which may be present in the residue. Any of such liquid slag or iron which tends to percolate downward into the mass will adhere as droplets to the solid particles of said mass relatively close to its surface portion, and, because of the lower temperature within the mass, may even solidify. However, such slag and iron so percolating will be returned to the surface portion of the mass by the incoming charge and there be remelted. The zinc produced is in the form of a vapor which, together with the carbon monoxide and other gases formed by the reaction and heat, escapes upward from the free surface portion of the mixture. These escaping vapors and gases agitate the upper surface portion of the mixture and cause the excess coke, coal and other solid particles, with the slag and iron droplets adhering to them, to gravitate down the sloping surface to its lower edge portion for removal from the chamber. The zinc vapors and gases which escape upward from the mass may be discharged from the chamber into a condenser where they are cooled for condensing the vaporous zinc to liquid zinc.

In the above described operation the residue which reaches the lower edge portion of the sloping surface of the mass of charge, because it consists in effect of molten slag and iron mixed with a variable amount of solid particles to which the molten constituents adhere, is rather pasty or sticky and does not flow readily. This residual material however may be readily removed from the furnace, if not too much solid material is present in it, by causing it to be heated by the downwardly radiated heat, when it reaches the lower edge portion of the sloping sur-

face and when it is pushed by the feeding operation onto a portion of the hearth beyond the mass of charge, to render it sufficiently liquid or limpid to be tapped from the furnace.

The molten iron-copper matte mixture, as it is formed at the sloping surface portion of the mass of charge and particularly as it is rendered limpid on the portion of the hearth beyond the mass of charge, acts to scavenge the residue of any precious metal values present in the oxidized zinc ore charged into the furnace, such values going into solution in such mixture. After the iron-copper matte mixture and slag with the solid particles of the residue are tapped from the furnace the iron-copper matte mixture can readily be recovered by liquation and treated for recovery of those precious metals by any one of several methods used by those familiar with the art.

The oxidized zinc ore seldom contains less than about 2% iron in the form of iron oxide usually with a small amount of iron in the form of iron sulphide. The total amount of iron in these forms varies considerably and commonly runs as high as 14%. Sufficient iron oxide, or iron sulphide or other iron compound capable of being reduced to metallic iron by the carbon, will be contained in the charge in amount sufficient to produce enough metallic iron to take up sufficient copper sulphide satisfactorily to scavenge the charge of its precious metal values if the amount of iron chemically so contained in the oxidized zinc ore is about 1%. In the rare case of an oxidized zinc ore which does not contain enough iron oxide or other carbon reducible iron compound the deficiency may be corrected by adding a requisite amount of the same to the charge with the reaction carbon, or even adding chips of cast iron of high enough carbon content to be readily meltable.

Copper sulphide dissolved in the iron acts very markedly to augment its property of scavenging the charge of its precious metal values. The copper sulphide, it has been found, will give appreciable results in this respect when the copper contained therein is chemically at least about 0.1% of the oxidized zinc ore. Ordinarily the ore will contain at least that amount of copper in the form of copper sulphide. In the rare case of a zinc ore which is deficient in copper sulphide such deficiency can be corrected by adding it, or copper in the form of any of the other compounds or minerals above mentioned, to the charge when the coke or coal is added, or even by adding metallic copper which will be converted to copper sulphide by the residual zinc sulphide contained in the oxidized zinc ore and any sulphur contained in the coke or coal.

The particular size of the granular coke or other carbonaceous reaction material employed and of the oxidized zinc ore is by no means critical, satisfactory results being secured if the particles of maximum size will pass a one inch mesh screen, the bulk of the particles of course being much smaller down to what would constitute powdered reaction coke or coal and oxidized zinc ore. However, unless the oxidized zinc ore is porous in structure the rate of reaction will be substantially increased by crushing it somewhat more finely.

The temperature to which the surface portion of the charge is heated of course depends upon the amount of heat radiated downward upon it. From a commercial standpoint, significant amounts of zinc vapors will be produced when the surface portion of the charge is heated to about 1700° F. It has been found, however, that the maximum temperature to which the surface portion of the charge can be heated is in the neighborhood of 2300° F., any increased amount of heat radiated downward on the charge merely serving to speed up the reaction, the effect being analogous to that observed in boiling water which may be heated to a boiling point of definite temperature without any excess amount of heat raising its temperature but merely increasing the rapidity with which the water boils to form steam.

According to the present invention, preferably sufficient

excess heat is radiated downward on the charge to heat its upper free surface portion to this maximum temperature and cause the reaction to take place rapidly so as to secure in effect a flash reaction. The molten slag and iron will be produced at about 1950 to 2250° F., as likewise will be produced the molten copper sulphide which dissolves into the iron, and consequently these molten materials will be produced at the maximum temperature mentioned to which the surface portion of the charge is heated.

Because of the reaction being endothermic and the charge being fed substantially continuously to the hearth at the same rate as the charge is consumed by the reaction, and said charge being of low heat conductivity, the reaction is confined substantially to the sloping surface portion of the charge and the molten droplets fail to penetrate the charge to any substantial extent below said surface portion without solidifying, with the result that the charge remains loose and is readily substantially continuously forced to said sloping surface portion as it is fed to the hearth. Furthermore, as the melting points of these droplets are less than the temperature at which the reaction will occur, any droplets which tend to penetrate downward into the charge tend to solidify within the zone in which zinc vapors and gaseous reaction products are evolved, which vapors and products tend to agitate the charge as they escape upward therefrom and hence tend to move the droplets toward the high temperature surface of the charge where if they have solidified they are remelted.

It will be observed that by entering the charge into the furnace chamber at a point below the upper surface portion of the charge therein and heating said surface portion to a temperature well above the temperature at which the reaction would begin to occur results in a gradual preheating of the charge as it moves from its point of entry into the chamber toward said surface portion, so that the charge when it reaches said surface portion is in condition to facilitate the above explained rapid or

flash reaction occurring at said surface portion.

The amount of coke or coal mixed with the oxidized zinc ore charged to the reaction chamber, if the residue is to be removed from that chamber as a liquid containing little solid residue, may be from 5 to 30% in excess of that which will give the amount of carbon stoichiometrically necessary to reduce all zinc oxide and the necessary amount of iron oxide or other carbon reducible iron compound present. Ten per cent excess carbon in respect to that stoichiometrically necessary to reduce the zinc oxide, it has been found, ordinarily will give excellent results in regard both to reducing the zinc oxide and producing the necessary amount of iron. With these amounts of excess coke or coal the pasty residue collecting at the lower end of the upper sloping surface of the charge on the hearth may be rendered sufficiently liquid or limpid to tap that residue from the reaction chamber if such residue is heated from about 2200 to 2500° F., the exact temperature necessary depending upon the composition of the slag and upon the proportion of coke or coal particles present. However, the temperature at which the residue becomes sufficiently liquid or limpid for this purpose may to some extent be controlled by adding, according to common metallurgical practice, fluxing materials, such as burned limestone, to the charge for the purpose of reducing the melting point of the slag produced. If the amount of excess coke or coal is much increased beyond the percentages thereof indicated so much solid coke or coal particles will be mixed with the molten slag or iron in the form of droplets adhering to particles of coke or coal that it becomes increasingly difficult to render the residue sufficiently liquid or limpid to tap it from the reaction chamber, so that with such excess amount of coke or coal it becomes necessary to take the resulting pasty mass of particles from the chamber. In some cases, however, it may be desirable

not to render the residue liquid enough to tap it from the chamber but to rake it therefrom, especially if the oxidized zinc concentrate does not contain precious metal values to be recovered, and in such case about 80 to 125% excess coke or coal is preferably employed.

The apparatus illustrated by the accompanying drawings may be employed for practising the above described methods, the drawings showing several modifications of electric furnaces which may form part of said apparatus.

In the drawings:

Fig. 1 is a central longitudinal vertical section, on the line 1—1 of Fig. 4, of a furnace for practising the methods according to the invention;

Fig. 2 is a section on the line 2—2 of Fig. 1, this section line for convenience in following the drawings 15 also being applied to Fig. 4;

Fig. 3 is a section on the line 3—3 of Fig. 2, with parts omitted;

Fig. 4 is a more or less diagrammatic plan view of apparatus for practising the methods according to the 20 invention, with parts omitted;

Fig. 5 illustrates more or less schematically a modified form of furnace; and

Fig. 6 illustrates a fragment of a further modified form of furnace.

Referring to Figs. 1, 2, 3 and 4 of the drawings, the furnace comprises an open top casing 1 of sheet metal, preferably steel, having side walls 3, 5, 7 and 9 and a bottom wall 11 all welded together to form a fluid tight construction. As shown, this casing is provided with a cover 13 comprising a reinforced metal plate 15 the bottom surface of which rests on the upper edge of the side walls of the casing. The cover is removably secured to the casing by the bolts 17 welded at their lower end portions to brackets 19 (Fig. 2) secured to the stiffening bars 21 for the side walls 7 and 9 of the casing, to which latter the inner edges of these bars are welded. Extending continuously around the upper edge portions of the side walls of the casing 1 are angle-irons 23 the edges of the horizontal webs of which are welded to the casing side walls in a fluid tight manner to form a trough 25 which is filled with sand, oil or the like and into which projects a flange 27 extending continuously around the edge of the cover plate 15 at its under side in fluid tight welded relation thereto. In this way the cover is secured to the casing in a fluid tight manner.

Internally the casing 1 contains a structure which forms a furnace chamber having an upper portion 29 and a lower portion 31. The bottom of the lower portion 31 is built up of hard carbon blocks 33 to form a hearth 35, which hearth, as shown by Fig. 2, is of arcuate cross-section. The blocks 33, as shown by Fig. 1, extend from one end of the furnace chamber to a point spaced from its opposite end to form a well or pit 37 having a bottom wall 39 formed by the hard carbon blocks 41.

At opposite longitudinal sides of the hearth the blocks 33, as shown by Fig. 2, abut the wedge-shaped blocks 43 a row of which extends for the entire length of the chamber. On the upper flat surfaces of these wedge-shaped blocks are supported at opposite sides of the chamber the elongated horizontal graphite slabs 45, similar slabs of graphite 47 being positioned at opposite ends of the chamber. These slabs 45 and 47 are grooved at their upper sides as shown at 49, these grooves communicating with each other at the four corners of the chamber. The grooves in the slabs 45 receive the lower edge portions of vertically positioned horizontally extending graphite slabs 51, and the grooves in the slabs 47 receive the lower edge portions of vertically positioned horizontally extending graphite slabs 53, the slabs 51 and 53 abutting at the four corners of the chamber. Supported by each of the slabs 51 at their upper edges are graphite bars 55 which, as shown by Fig. 4, extend for the length of the chamber, while supported by each of the slabs 53 at their upper edges are graphite bars 57

which extend for the transverse width of the chamber, the bars 55 and 57 abutting adjacent the four corners of the chamber and being grooved at their lower sides, as shown at 59, for receiving the upper edges of the slabs 51 and 53. Resting on the upper sides of the bars 55 are vertically positioned horizontally extending graphite slabs 61, while resting on the bars 57 are vertically positioned horizontally extending graphite slabs 63, these slabs 61 and 63 abutting each other at the four corners of the chamber, and the upper sides of the bars being grooved, as shown at 65, for receiving the lower edges of the slabs. The roof of the chamber is formed by the laterally abutting elongated graphite slabs 67 which rest at their opposite end portions on the top edges of the slabs 61, the edge portions of the slabs 67 adjacent the slabs 63 also resting on the top edges of the latter.

The carbon blocks 33 and 41 forming the hearth 35 and the bottom wall 39 of the well or pit 37, respectively, are supported on a layer formed by courses of firebricks 69, which layer at the sides of the wedge-shaped blocks 43 and adjacent the longitudinal ends of the casing 1 is built upward to support and back the slabs 45 and 47 and to form firebrick layers 71 adjacent the side walls of the casing. On the tops of the firebrick layers 71 rest the elongated graphite slabs 73 which close the space surrounded by said layers. The space between these slabs and the furnace chamber roof slabs 67, and the space between the firebrick layers 71 and the slabs and bars forming the interior side walls of said chamber, are filled with a mass of heat insulating material 75 as, for example, carbon beads or a mixture of the same and lamp black or broken up charcoal.

Between the slabs 73 and the cover 13 of the casing 1, and between that casing and the firebrick layers adjacent its sides and bottom, are inserted heat insulating packing layers 76 of material capable of resiliently yielding under high pressure to permit the furnace casing and the interior walls of the furnace to expand and contract independently of each other so as to prevent rupture of the casing.

In the upper portion 29 of the furnace chamber is positioned a row of parallel elongated heating resistor bars 77 preferably of graphite. The opposite end bars of the row have extensions 79 projecting through the furnace walls in electrically insulated relation thereto, and at the exterior of the furnace these two extensions are provided with terminals 81 for the cables for energizing the resistors, the resistors being connected at opposite ends for series flow of current through them. The resistors are supported from the roof slabs 67 by the elongated graphite bars 83, which latter are carried by said slabs in electrically insulated relation thereto. The construction of the resistors and their suspension is more fully described in Poland United States Patent 2,472,613, issued June 7, 1949, and in pending United States application of Richard 55 A. Wilkins, Serial Number 162,220, filed May 16, 1950, and need not be further described here. The resistors when heated become incandescent and radiate heat downward toward the hearth. They also act to heat the graphite roof of the chamber to incandescence to cause it also to radiate heat downward toward the hearth.

As shown, interposed between the resistors and the hearth is a row of laterally abutting elongated bars 85, of circular cross-section, formed of graphite which is extremely heat refractory and an excellent conductor of heat. These bars form a partition dividing the furnace chamber into its upper and lower portions 29 and 31. They serve to protect the resistors from attack by dust, vapors and gases emanating from the heated charge. The circular cross-section of the bars gives the upper and lower sides of this partition a corrugated shape which increases the area of those sides and therefore increases the facility with which the partition absorbs the heat from above and radiates such heat downward toward the hearth.

As shown, the bars 55 are formed to provide shelves 75 87 on which the ends of the bars 85 rest, these shelves

being inclined downward from one bar 57 to the other so that when the bars 85 are placed on the higher ends of the shelves they will roll downward to the lower ends of the shelves and there rest against the abutments 89 formed by the bars 57 at said lower ends. The bars 85 may be inserted and removed from the furnace without cooling it. For this purpose the walls of the furnace are provided with openings in one of which adjacent the higher end of the inclined shelves 87 is positioned a graphite sleeve 91 (Fig. 4), and in another of which adjacent the lower end of those shelves is positioned a graphite sleeve 93. These sleeves are received at their inner ends in the enlarged diameter portions 95 of openings 97 in the adjacent bar 55. The sleeves are normally plugged with removable stoppers in the form of bars 99 preferably of hard carbon which is a relatively poor heat conductor, these bars being preferably of such length as to extend for the full length of the sleeves so as to minimize heat losses from the chamber. As shown, those ends of the sleeves 91 and 93 which project from the outer side of the furnace are surrounded by the water jacketed metal sleeves 100 welded at one end to the casing 1, which sleeves 100 keep the outer ends of the carbon bars 99 cool enough to be conveniently handled. Upon removal of the plug from the sleeve 93 the bar 85 at the lowermost ends of the inclined shelves 87 may be pushed out of the furnace through such sleeve by means of a metal rod inserted and pushed through the graphite sleeve 101 of small diameter bore positioned in an opening in the furnace wall opposite the sleeve 93 in alignment therewith, this sleeve 101 communicating with an opening 103 formed in the adjacent bar 55. The bore of the sleeve 101 may be normally plugged with a stopper in the form of a carbon bar similar to one of the bars 99. Ordinarily however, due to the small diameter of the bore of the sleeve 101, it will suffice if such bore is closed by a metal cap 105 screw-threaded on or otherwise removably carried by a metal sleeve 107 which surrounds the outwardly projecting end of the sleeve 101 and is welded to the adjacent wall of the casing 1. For supporting the bars 85, when they are being inserted and removed from the furnace chamber, the bars 57 are each formed with a shelf 109 on which the bars slide for preventing them from tilting and falling downward into the lower portion of the furnace chamber. It will be understood that upon removal of a bar 85 at the lower ends of the inclined shelves 87 the remaining bars will roll down said shelves to place the next consecutive bar 85 opposite the sleeve 93 and thus leave a space at the higher ends of such shelves into which a new bar may be inserted through the sleeve 91 when the stopper bar 99 in that sleeve is removed.

As further shown, the furnace according to Figs. 1, 2, 3 and 4 is formed with a tap hole 111 communicating with the well or pit 37, this tap hole being normally closed by a removable plug 113 of fireclay or the like, upon removal of which the material in the well may be tapped therefrom as a liquid mass or be raked therefrom depending upon the temperature of such mass and the amount of solid particles contained therein.

Also, preferably, the exterior of the casing 1 at its lower portion is surrounded by a water jacket 115 which has the effect of cooling the exposed surfaces of the hearth and well 37 so that there will be formed thereon a rather thin layer of solid iron or slag or a mixture of the two, the iron usually being in the form of magnetite. This layer protects the carbon blocks forming those surfaces from destruction by the molten iron, which tends to dissolve them, and by the residual zinc oxide dissolved or mixed in the slag, which zinc oxide tends aggressively to react with them. The iron and slag have about the same melting point, although the same may vary somewhat with each depending upon its exact composition. The cooling effect of the water jacket is so coordinated with the thickness and heat conductivity of the materials forming the adjacent portion of the furnace walls that when molten slag or iron contacts the sur-

faces of the hearth and well it will solidify and its thickness increase until its surface temperature reaches the melting point of the slag or iron, whereupon the protective layer thus formed will not build up farther, or, if the slag or iron when it first contacts these surfaces of the hearth and well eats them away, the consequent slight thinning of the blocks presenting those surfaces will cause such surfaces to reach a temperature which will solidify the slag or iron contacting them, which solidified slag or iron will build up to form a protective layer until the thickness of such layer is such that its exposed surfaces are at their melting points.

In the above connections it will be understood that in operation normally only the well 37 and the portion of the hearth at the left of the charge as viewed in Fig. 1, and its portion below the charge adjacent the lower end of the upper sloping surface of the charge, will be subjected to the form of destruction mentioned as its portions well beneath the charge will, because of the heat insulating effect of the charge, be ordinarily cool enough to prevent liquid slag or iron from reaching them. However, the hearth throughout its entire length will tend to be subjected to such destruction when initiating the charging operation with a preheated furnace, and consequently the water jacket preferably surrounds the entire lower portion of the furnace.

As shown, the vertical wall of the furnace adjacent the end of the hearth opposite the well 37 comprises a sleeve 117 of hard carbon having a tapered bore 119. At its outer end this bore is provided with a metal sleeve extension 121 communicating with the horizontal conduit 123 (Figs. 1 and 4) at the exterior of the furnace. This conduit communicates at one end with the bottom discharge opening 125 (Fig. 4) of a hopper 127, which opening is provided with a gate valve 129, shown in partly closed position in Fig. 4, so that the conduit 123 can be closed when desired. Extending lengthwise of the interior of the conduit is an elongated rotary screw conveyor 131 schematically shown as driven by an electric motor 133 through a reduction gear (not shown) contained in a casing 135. The mixture of oxidized zinc ore and coke or coal is entered into the hopper so as to discharge into the conduit 123 through which the screw conveyor forces the material and causes it to pass through the bore 119 to feed such material to the furnace and form on the hearth a pile or mass 137 (Fig. 1) having a downwardly sloping free upper surface 139 the slope of which is determined by the angle of repose of the material. This material builds up at its higher end to above the bore 119, and the incoming material from said bore acts to force the material toward the sloping surface of the pile substantially throughout the entire extent of said surface and to move the residue at the lower end of the pile along the hearth in a direction which is away from said bore.

The heat radiated downward on the upper sloping surface of the mass of charge will cause, in the way hereinbefore described, solid particles of the excess coke or coal and other residue with adhering droplets of molten slag and iron to gravitate down the sloping surface of the mass of charge to the lower edge portion of said mass, while the incoming charge will cause such particles with the adhering droplets to be pushed on the portion of the hearth beyond the lower edge of said sloping surface. On such portion of the hearth, if there is not too much excess of coke or coal and other solid residue, the heat radiated downward on that portion will render this slag or iron sufficiently liquid or limpid to flow into the well or pit 37 and carry with it such excess coke or coal and other solid residue, from which well the material may be tapped through the tap hole 111, as hereinbefore described. If there is a large excess of coke or coal the same with the adhering slag or iron droplets will build up on the portion of the hearth just mentioned and work toward the edge of the hearth

and fall into the well as a sticky or pasty mass which can be raked from the well through the tap hole.

As shown, the hearth is provided with a bore 141 (Fig. 1) leading to the exterior of the furnace. In this bore is removably inserted a tube 143 having a thermocouple at its outer end 145, leads 147 from the thermocouple extending through the tube to the exterior of the furnace being connected to a suitable instrument (not shown) for indicating the temperature of the thermocouple. For a given amount of heat radiated downward on the charge, and a given thickness of the portion of the charge above the thermocouple, the thermocouple will indicate a definite temperature, this temperature being normally somewhere about 1900° F. if the thermocouple is, as shown by Fig. 1, positioned beneath the charge near the lower end of its upper sloping surface and sufficient heat is radiated on the charge to secure the flash reaction hereinbefore described. The thermocouple may, if desired, be placed under a thicker portion of the charge where because of the heat insulating effect of the charge the temperature of the hearth will be lower, but best results it has been found will be secured by placing it under the charge near the lower end of the upper sloping surface of the charge. By observing the temperature indicated by the thermocouple when satisfactory operation is secured, and maintaining a rate of feed of the charge to the furnace to keep that observed temperature approximately constant, such satisfactory operation will be continued if the amount of current flowing through the resistors is kept constant.

The vaporous zinc admixed with the gaseous products of the reaction escape from the furnace chamber through an opening 149 in the furnace wall, from which opening they are led through a conduit 151 to a condenser 153 (Fig. 4) where the vaporous zinc is condensed to liquid zinc, the gaseous products escaping from the top of the condenser through a stack 155 provided with a damper 157 which may be adjusted to regulate the pressure within the condenser and furnace chamber. Normally satisfactory results will be secured with a pressure in the furnace chamber and condenser just slightly above atmospheric. So maintaining the pressure prevents leakage of air into the furnace chamber and condenser through any possible interstices in their walls as well as through the charging opening 119. It also prevents air from entering the furnace chamber when the tap hole 111 is opened for discharging liquid residue from the well or pit 37 or for raking sticky or pasty residue therefrom. Conveniently, when such residue is to be removed from the well, the energy input to the resistors is temporarily reduced to decrease the evolution of zinc vapors from the charge so as to decrease the amount of the same that might escape from the furnace chamber through the tap hole when it is opened, the damper 157 being adjusted, if necessary, when the tap hole is opened to insure that the pressure within the furnace chamber remains slightly above atmospheric.

Maintaining the mass of charge on the hearth adjacent the bore 119 well above that bore, as shown in Fig. 1, acts to insulate the material in that bore and that portion of the material on the hearth which is adjacent the discharge end of said bore from the downwardly radiated heat so that no substantial reaction between the zinc oxide and carbon will occur in such material so insulated. If it did occur the zinc liberated would tend to condense at the cooler portions of the bore and tend to clog it. For further insuring that no reaction of the zinc oxide and carbon will occur in the bore 119 the portion of the water jacket 115 at the end of the furnace adjacent that bore is extended upward to form a portion 158 that surrounds the sleeve extension 121 of the bore, and by absorbing heat from the adjacent portion of the furnace walls acts to keep the material in said bore and extension at a temperature below that at which any substantial reaction between the zinc oxide and carbon oc-

curs. For preventing zinc vapors from being forced from the furnace chamber through the charge into the bore 119 and charging conduit 123, and into said bore and conduit when the charge is being initially entered into the preheated furnace or when the mass of charge on the hearth is otherwise at a low level, in which bore and conduit such vapors would condense to troublesome solid metallic zinc and interfere with the charging operation, the block or sleeve 117 is shown as formed with a passage 159 (Fig. 1) which opens into the bore 119 of said block. Through this passage an inert gas, such as nitrogen, may be fed to the bore 119 from a supply pipe 161 communicating with said passage, the flow of nitrogen being controlled by a valve 163 in said pipe. The amount of nitrogen so admitted to the bore 119 may be regulated by the valve to cause the pressure in that bore to be slightly higher than that in the furnace chamber so as to prevent backflow of the zinc vapors into said bore and the conduit 123. Nitrogen from this passage may also be admitted to the furnace chamber and hence to the condenser for displacing the air contained in them prior to heating the resistors and furnace chamber preliminary to initiating the smelting operation.

If desired, the furnace chamber may be fed with charge from each of opposite ends of the hearth as schematically illustrated in Fig. 5, in which case the well or pit 37 may be positioned midway the length of the hearth, two sets of resistor bars 77, and bars 85 for protecting said resistors, preferably being provided in such case.

In the practice of the method as hereinbefore described the residue may be rendered sufficiently liquid or limpid to tap it from the furnace if the excess amount of coke or coal is small, whereas if such excess is large the residue will not be so rendered and must be raked or the like from the furnace in the form of a more or less sticky mass of substantially solid particles. However, by use of the furnace according to Fig. 6, the residue in its last mentioned form may be raked from the furnace when employing the smaller amounts of excess coke or coal, it being understood that it may be of advantage to perform the method in this way when the oxidized zinc ore does not contain precious metal values or it is not economically feasible to recover them. Employing the smaller amount of excess coke or coal of course effects a considerable saving in these materials, while not heating the residue sufficiently to render it flowable conserves heat energy.

The furnace according to Fig. 6 is identical with that shown by Figs. 1, 2, 3 and 4 except that the well or pit 165 of that according to Fig. 6 is deeper and wider than the well or pit 37 of that according to Figs. 1, 2, 3 and 4. Above the well 165 the adjacent side wall of the furnace is provided with elongated carbon blocks 167, 169 and 171 which project from said well to form a shield above the well and the adjacent extreme end portion of the hearth 35 to shade the well and that portion of the hearth from the downwardly radiated heat. This shading of the well and adjacent portion of the hearth insures that the residual material in the well and on that portion of the hearth will not be heated to a high enough temperature to make the slag and iron sufficiently liquid or limpid to permit the residue to be tapped from the well, the residue in this case being raked from time to time from the well through the normally plugged hole 111 in the form of a more or less sticky mass of solid particles. To enable the residue to be raked from the well or pit 165, when using the furnace according to Fig. 6, the mixture of oxidized zinc ore and coke or coal is fed to the furnace chamber at such rate as to maintain on the hearth a mass having an upper downwardly sloping surface 173 the lower edge 175 of which is at the portion of the hearth shaded by the above described heat shield so that the residue on the hearth and in the mass of charge adjacent the edge 175 will not be heated sufficiently to make it liquid or limpid and will be pushed off the hearth and fall into the well or pit 165 in the form of the above mentioned more

or less sticky mass of solid particles. The material in the well, being effectively shielded from the downwardly radiated heat, in some instances will further cool to substantially solidify the liquid or pasty droplets of slag and iron adhering to solid particles of the residue so that adjacent the hole 111 as the residue accumulates in the well such residue will be more or less in the form of a dry mass of granular particles.

In all instances of the practices of the methods described the charge may be fed to the furnace chamber substantially continuously as an uninterrupted stream, or as an intermittently flowing stream, or in batches each constituting a relatively small fraction of the charge on the hearth, so long as the overall rate of feed is such that it substantially equals the overall rate at which the charge is consumed by the reaction and a mass of charge having an upper sloping surface and a portion above the level of the charging port is maintained on the hearth during the continuance of the smelting operation. It will also be understood that specific feeding means herein disclosed constitutes in substance a form of under feed stoker and that other suitable forms of under feed stokers may be substituted for it.

Other oxidized zinciferous substances have compositions analogous to that of the roasted or oxidized zinc sulphide ore concentrates above described in that they contain zinc oxide, iron or carbon reducible iron compound and slag forming materials, and, in some instances, copper sulphide or mineral or compound which in the presence of zinc sulphide or sulphur in the charge will cause copper sulphide to be formed, and also, in some instances, precious metal values. Among these are naturally occurring oxidized zinc ores and concentrates of the same, so-called "densified zinc oxide," the residue of conventional zinc retorts, galvanizing dross, the waste products of lead smelters, certain zinc dusts, and other zinciferous residues, drosses, slags, dusts, wastes and secondary materials. These other oxidized zinciferous substances may be treated, according to the present invention, in the same way as the roasted or oxidized zinc sulphide ore concentrate by crushing them to render them granular when they are not already in suitable powdered or otherwise granular form, and mixing them with granular reaction carbon when they do not already contain the same or contain an insufficient amount thereof, sufficient copper sulphide or substance that will form copper sulphide in the way hereinbefore described also being added, if necessary, to enable the precious metal values to be recovered if such values are present and it is desired to recover them. Other oxidized zinciferous materials which do not in themselves contain slag forming material or iron may also be treated according to the invention by rendering them granular by crushing them, or, if in very finely divided form, by balling or briquetting them and, if necessary, crushing the balled or briquetted material to secure the desired granule size, after which the granular material is mixed with granular reaction carbon to form the charge, iron or carbon reducible iron compound and copper sulphide or the like being added only if the material contains precious metal values that it is desired to recover.

For convenience in terminology, in the appended claims the oxidized zinc sulphide ore concentrate and other oxidized zinciferous substances above mentioned are referred to generically as "zinciferous material containing zinc oxide," while copper sulphide and the copper compounds, copper bearing minerals and added metallic copper which cause copper sulphide to be formed in the way hereinbefore described (so that their presence causes the zinciferous material or mixture of the same and reaction carbon in substance to contain copper sulphide) are referred to generically as "copper sulphide."

In the above connections it will be understood that the presence of slag forming materials in the charge is not essential to the recovery of the zinc, or to the removal

of the residue from the furnace chamber unless it is desired to remove it therefrom as a liquid containing the solid particles, although as a practical matter slag forming materials always will be present if coke or coal of usual composition is employed to present the necessary reaction carbon, and, of course, iron and copper sulphide are not necessary if the zinciferous material contains no precious metal values or it is not desired to recover them. In any rare case where it may appear necessary slag forming materials may be added to the charge to enable the residue to be tapped in such liquid form.

It will be also understood that within the scope of the appended claims wide deviations may be made from the forms of methods, apparatus and furnaces described, without departing from the spirit of the invention.

We claim:

1. The method of smelting zinciferous material containing zinc oxide and slag forming constituent which comprises feeding a granular mixture of such material and reaction carbon to a hearth in an operatively closed chamber at such rate as to maintain continuously on said hearth during the continuance of the smelting operation a mass having an upper surface sloping downward to adjacent an edge portion of said hearth; radiating heat downward from above said mass, while shielding the portion thereof adjacent said edge portion of the hearth from such heat, to react the zinc oxide and the carbon at the upper surface portion of the unshielded part of said mass to liberate vaporous zinc from such portion and melt slag forming constituent of said surface portion to cause molten slag admixed with solid particles of the residue to gravitate down said sloping surface to the shielded part of said mass; removing the slag and residue mixture from said hearth in non-liquid condition, and discharging the vaporous zinc from said chamber.

2. The method according to claim 1 in which the mixture is fed to the mass of charge on the hearth from beneath the sloping surface of said mass adjacent the higher portion of said surface.

3. The method of electrothermically smelting zinc from a mixture containing zinc oxide, excess reaction carbon, and slag forming substance, which comprises feeding such mixture in granular form to a hearth in an operatively closed chamber at such rate as to maintain continuously on such hearth during the continuance of the smelting operation a mass having an upper surface which slopes downward to said hearth at an edge portion of said mass at an inclination determined substantially by the angle of repose of such granular mixture; continuously heating the sloping upper surface portion of said mass during the continuance of the smelting operation by heat caused to be radiated upon it by electric heating resistors positioned above said hearth and mass to react at said surface portion zinc oxide and carbon of said mixture for forming vaporous zinc and gaseous reaction products, the latter consisting mostly of carbon monoxide, and for forming slag which adheres to solid particles of the residue of the mixture at said surface portion; said vaporous zinc and gaseous reaction products filling said chamber and being discharged therefrom for condensation of the vaporous zinc; the heat radiated downward on such surface portion being of such intensity as to cause said vaporous zinc and gaseous reaction products while escaping from said surface portion to agitate it to cause such solid residue and adhering slag to gravitate down said sloping surface portion to the portion of the hearth at the lower edge portion of said surface portion where it is received by the hearth as a pasty mass; substantially continuously removing from said portion of the hearth, to a heated portion of said chamber below the level of said edge portion of said sloping surface portion, the residue and slag so caused to be received by the hearth for keeping such slag out of contact with said mass of mixture on the hearth; and from time to time as said slag accumulates in said heated por-

**13**

tion of the chamber removing it and such of said residue as remains with it from said chamber.

4. The method according to claim 3 in which the granular mixture is fed to the mass of mixture on the hearth at such position below the sloping surface portion of said mass as to force the mixture toward said surface portion substantially throughout the extent of said surface portion for causing the incoming mixture to reach said surface portion in preheated condition, and for causing the slag and residue gravitating down said surface portion to the hearth to be pushed over said hearth away from said mass. 10

5. The method according to claim 3 in which the heat radiated toward the hearth at the portion thereof which receives the pasty mixture of residue and slag that gravitates down the sloping surface portion of the charge on the hearth is sufficient to render that mixture sufficiently limp while on the hearth to cause it to flow to that heated portion of the chamber which is below the level of the adjacent portion of said charge. 20

6. The method according to claim 3 in which the heat radiated toward the hearth at the portion thereof which receives the pasty mixture of residue and slag that gravitates down the sloping surface portion of the charge on the hearth is sufficient to render that mixture sufficiently limp while on the hearth to cause it to flow to that heated portion of the chamber which is below the level of the adjacent portion of said charge, and said heated portion of said chamber is maintained at such temperature as will maintain said mixture in such limp condition. 25 30

7. The method according to claim 3 in which the

**14**

granular mixture fed to the hearth also contains carbon reducible iron compound, copper sulphide, and precious metal, the heat radiated on the sloping surface portion of said mixture being sufficient also to react the carbon with such iron compound to form molten iron for dissolving copper sulphide of said mixture, which iron also adheres to the residue of said mixture and gravitates with said residue and slag to the hearth; heating the pasty material so gravitating to the hearth while on the hearth to render it sufficiently liquid to cause the iron-copper sulphide solution to scavenge the residue of its precious metal values and to flow to that heated portion of the chamber which is below the level of the edge portion of the charge on the hearth, the temperature of said heated portion of said chamber being sufficient to maintain said material flowing to its liquid, and upon removal of said material from said chamber treating it to recover the precious metal values so scavenged. 15

**References Cited in the file of this patent****UNITED STATES PATENTS**

|           |                  |       |                |
|-----------|------------------|-------|----------------|
| 1,516,651 | Tharaldsen       | ----- | Nov. 25, 1924  |
| 1,647,279 | De Saulles       | ----- | Nov. 1, 1927   |
| 2,144,914 | Debuch           | ----- | Jan. 24, 1939  |
| 2,377,478 | Bowen            | ----- | Jan. 5, 1945   |
| 2,473,611 | Robson           | ----- | Jan. 21, 1949  |
| 2,482,445 | Turner           | ----- | Sept. 20, 1949 |
| 2,598,743 | Waring et al.    | ----- | June 3, 1952   |
| 2,598,745 | Handwerck et al. | ----- | June 3, 1952   |